

Dec. 7, 1948.

G. D. RECHTON ET AL.

2,455,702

## METHOD OF FORMING MATERIAL

Original Filed Sept. 7, 1942

2 Sheets-Sheet 1



GEORGE D. RECHTON  
DELBERT J. WARD  
JACK H. WATSON  
INVENTORS

BY *Edwin Coates*  
ATTORNEY

Dec. 7, 1948.

G. D. RECHTON ET AL

2,455,702

## METHOD OF FORMING MATERIAL

Original Filed Sept. 7, 1942

2 Sheets-Sheet 2



## INVENTORS

GEORGE D. RECHTON  
DELBERT J. WARD  
JACK H. WATSON  
BY

BY

BY  
*Edwin Coates*  
ATTORNEY

## UNITED STATES PATENT OFFICE

2,455,702

## METHOD OF FORMING MATERIAL

George D. Rechton, Los Angeles, Delbert J. Ward, Sherman Oaks, and Jack H. Watson, Los Angeles, Calif., assignors to Douglas Aircraft Company, Inc., Santa Monica, Calif.

Original application September 7, 1942, Serial No. 457,630, now Patent No. 2,372,516, dated March 27, 1945. Divided and this application September 20, 1944, Serial No. 555,028

7 Claims. (Cl. 153—21)

1

This invention relates to a method of forming bodies of metal and other materials, and more particularly to a method for forming sheets of magnesium alloy and other metals having qualities which prevent their being formed at ordinary temperatures without the development of structural weaknesses. The present application is a division of our copending application Serial No. 457,630, filed September 7, 1942, now U. S. Patent No. 2,372,516.

The word, form, as used herein means any processing operation which establishes and changes the shape or dimension of an article or divides the article into a plurality of articles such as bending, punching, blanking, stamping, and shearing.

The aircraft industry, in line with the trend toward lighter and faster aircraft, has been steadily increasing the use of metals having low specific gravities such as magnesium. Although magnesium ranks eighth in abundance among the elements of the earth, it has not been used extensively in any industry until the last few years. The slow adoption of this element in industry has been due in a great degree to difficulties in perfecting economical and practical methods of processing the same.

There have been many attempts to cold form sheets of industrial magnesium alloys characterized by structural strength but these attempts have not met with any noteworthy success. For example, it has been found that when it was attempted to dimple sheets of magnesium alloys that incipient fractures would appear adjacent the sharp radius bends formed at the base of the dimple. These fractures indicated structural weakness which made the sheet undesirable, particularly for use in aircraft construction.

Research and experimental work has shown that by heating the sheets of magnesium alloys to an ascertained temperature, for example, in the case of one magnesium alloy, to approximately 700° Farenheit, these metals can be dimpled or otherwise formed without the occurrence of fractures. Following this discovery several methods were proposed to raise the temperature of the sheet before the same was formed, but these previously proposed methods, for several reasons, proved unsatisfactory.

One method previously proposed consisted in heating the sheet electrically by passing a current therethrough using the dimpling dies as electrodes in a manner similar to that followed in the spotwelding process. This method was unsatisfactory as it caused the dimpled metal and

2

the dies used to become pitted from excessive arcing which took place because of the insulating qualities of the surface protecting coat on the magnesium sheet. This difficulty, coupled with excessive heating and consequent softening and deformation of the dies, rendered the machine for this method of heating impractical and expensive to operate.

In order to avoid these undesirable results this invention contemplates the provision of a method in which there is employed a heating means which does not involve excessive heating of the forming dies, and does not involve transmitting currents of electricity through the dies or other electrodes and the sheet of material being worked upon. The preferred form of the apparatus which can be used for carrying out the method of the present invention embodies a means for heating the sheet and dimpling the same while the sheet is maintained in the heated condition.

Two electric heat elements are provided on the machine shown, and the sheet to be dimpled is mounted intermediate the same. The elements when heated are brought into contact with the upper and lower faces of the sheet to secure an even distribution of heat throughout the area to be dimpled. The area to be dimpled should be raised to a temperature in excess of the temperature at which the metal will yield under pressure along both the pyramidal and basal planes without fracture, but less than the temperature at which the metal when subjected to a minimum effectively sufficient flexural forming pressure, will be appreciably thinned or will be caused to flow appreciably. With the area heated to a temperature within this range the metal may be successfully formed if a pressure is used which is sufficient at the particular temperature to which the metal is heated to form the metal but not so high as to appreciably thin the metal or cause it to flow.

In the preferred embodiment of the method of the present invention, the heating elements are first placed in close proximity to the area to be dimpled but held out of contact therewith until the area is preheated, after which the heat elements are moved into contact with the opposite surfaces of the sheet. After the area to be dimpled has reached the predetermined ascertained temperature the area is formed or dimpled by forming tools. The heating element adjacent the area to receive the maximum pressure is held at a temperature higher than the other element. The area adjacent the heating element having the highest temperature is not excessively heated

for in the highest range of temperature the area to be dimpled actually has a temperature only slightly in excess of that of the cooler element as heat is subtracted from the sheet by the cooler element.

Other features and advantages of the method of the present invention will be apparent from the following description taken in connection with the accompanying drawings in which:

Figure 1 is a side elevation of one form of a dimpling machine which can be used to carry out the method of the present invention;

Figure 2 is a front elevation of the machine shown in Figure 1; and

Figure 3 is a schematic view showing the dimpling device, the pneumatic mechanism for their operation, and a wiring diagram of the electrical equipment for the heating elements for control of the pneumatic equipment and for performing other functions in the operation of the machine to carry out the method of the present invention.

While the method of the present invention may be carried out by any suitable mechanism desired a dimpling machine has been selected to illustrate one machine which can be used to perform the method.

Figures 1 and 2 show a dimpling machine 10 having a base 11 upon which is mounted a supporting column 12. A pair of generally horizontal laterally extending arms 13 and 14 are clamped to the column 12, the upper arm 13 supporting at its outer end a pneumatic tool operator 15 and the lower arm 14 supporting at its outer end a lower dimpling anvil assembly 16.

The tool operator 15 is mounted for vertical movement in the guide 18 at the outer end of the upper arm 13 by a lever 19 which is fulcrumed at 21 between ears 22 extending upwardly from the upper arm 13 and which is connected at its outer end to the upper end of the tool operator 15 at 23 and is connected at its inner end to a piston rod 24 of a piston 25, shown only in Figure 3, operating within a pneumatic cylinder 26 mounted upon the rear end of the upper arm 13. The lever 19 is spring loaded by a spring 27 compressed between a stationary lug 28 and a collar nut 29 on a bolt 31 which passes through an eye in the lug 28 and is pivoted at its outer end to the free end of a depending arm 32 on the lever 19. As the spring 27 tends to move the left end of the lever 19 downwardly as viewed in Figure 1, a stop bar 33 is mounted on the arm 13 to engage the under side of the rear end of the lever 19 to prevent the piston 25 from striking the bottom of the cylinder 26.

The lower end of the tool operator 15, carries a forming tool or female die 34 and is surrounded by a heating element or heating body 35 of annular form. The heating element 35 is held in position laterally with respect to the tool operator 15 and supported vertically by a piston 36 which is vertically reciprocably movable within a pneumatic cylinder 37 mounted upon the outer end of the upper arm 13 adjacent the inner side of the tool operator 15. Admission of air to the pneumatic cylinder 37 moves the heating element downwardly and upon exhaust of air from this cylinder, the heating element is retracted to its normal position by the action of a tension spring 38 secured at its upper and lower ends to the guide 18 and piston 36 respectively. A cable 39 contains the electrical conductors for heating the element 35 and registering its temperature.

To the upper face of the outer end of the arm

14 is secured a pneumatic cylinder 40 to which air is supplied at an inlet 41 in which reciprocates a tubular piston 42, schematically shown in Figure 3, which carries at its upper end a heating element or heating body 43 which is apertured for the accommodation of the stationary male dimpling die 16. The support for the die 16 extends downwardly through the hollow piston 42 and is mounted upon the lower arm 14. The heating element 43 is thus vertically slideable with respect to the stationary dimpling die 16 from a lower retracted position to an upper position in which it makes contact with the metal sheet to be dimpled. A cable 44 contains the conductor wires for supplying the energy to heat the heating element 43 and to register its temperature.

A microswitch 45 closed upon downward movement of the heater 43 to its lower retracted position, is connected to the control mechanism by a cable 46, the cables 44 and 47 entering a junction box 48 from which electrical connections are made to the control and indicating devices by a cable 49.

The system of air conduits and pneumatic control devices for operation of the pneumatic cylinders 26, 37 and 40, and for operation of the pneumatic cylinder 51 of the tool operator 15, are shown schematically in Figure 3, some of the conduits and control devices appearing in the structural views, Figures 1 and 2. Air enters the machine under pressure at 52 through a gate valve 53 and may proceed to an electrically controlled valve 54 through the pipe 55 and thence, when valve 54 is opened, through a pipe 56 to cylinder 26 to actuate the lever 19 to depress the tool operator 15.

Air may also pass from the gate valve 53 to the electrically controlled valve 57 through pipe 58, for transmission when valve 57 is in the open position through supply conduit 59, and then pipes 60 and 61 to cylinders 37 and 40 respectively for movement of the heating elements 35 and 43 respectively from their retracted position to their position of contact with the metal sheet to be dimpled. Electrically controlled exhaust valves 62 and 63 are in closed position when valves 54 and 57, respectively, are in open position, and vice versa. The function to relieve the air pressure in cylinder 26 and in cylinders 37 and 40 respectively for the elevation of the tool operator 15 in the case of cylinder 26 and the retraction of the heating elements 35 and 43 in the case of the cylinders 37 and 40.

A valve 64 and a pressure gauge 67 in the supply conduit 59 communicating with the T connection 66 joining the supply conduit 59 with pipes 60 and 61, provide means for regulating the air pressure transmitted to cylinders 37 and 40 at any desired value, thus regulating the degree of pressure at which the heating elements engage the metal sheet. The section of exhaust pipe in which exhaust valve 62 is placed, the air supply pipe 55 and the pipe 56 leading to the cylinder 26 are connected as shown by a T 68. The exhaust pipe in which valve 63 is placed, the air supply pipe 58 and the conduit 59 leading to the T 66 are connected as shown by means of a T 69.

To T 71 interposed in the air supply pipe 55 is connected a pipe 72 leading to a pressure regulating valve 73, which in conjunction with a pressure gauge 74 serves to regulate the air pressure in pipe 75 leading to the cylinder 51 of the tool operator 15 and tripping the pneumatic firing device for applying an impulse force to the dimpling die 34 when the pressure between the upper

and lower dimpling dies reaches a prescribed value after the tool operator has been lowered and the two dies brought into engagement with the metal sheet to be dimpled, through depression of the tool operator due to actuation of the piston 25 operating in cylinder 26.

Upon an angle support 16 secured to the upper arm 13 is mounted a control box 77 which houses the electrical control equipment for the supply of current to the heaters 35 and 43 for sequential control of the electrical devices for the actuation of valves 54, 62, 57, and 63. These devices and their connections are enclosed within dash lines on Figure 3 and designated by the numeral 78. The valves 54, 62, 57, and 63 are electrically actuated by solenoids in a manner to be hereinafter explained, the conductors from the control box 77 to the various valve operating solenoids passing through a connection box 79 mounted on the inner end of the upper arm 13.

The front face of the control box 77 serves as a control panel 81 upon which are mounted the several dial switches and other manual controls, and the value registering instruments for use in operating the machine. These several control devices and registering instruments will be referred to and described in the course of the following explanation of the wiring diagram of Figure 3. On this diagram the arrows indicate the direction of potential drop.

Electrical energy is supplied to the control box by lead-in conductors 82 and 83. A warning light 84, connected across these main conductors 82 and 83, is placed on the panel to indicate passage of current to the control devices of the control box and thence to the heating elements and electrically operated valves. A line switch 85 controls the supply of current to the machine. Conductors 86 and 87 constitute a shunt heating circuit connected to the wires 82 and 83 of the power circuit, and supply electrical energy through a transformer 88 to the heating elements 35 and 43 in parallel through wires 89 and 91. The transformer 88 is of the variable tap type and includes an adjusting knob 92. The transformer controls the wattage input and consequently the temperature of the heaters 35 and 43. The primary of the transformer 88 is connected to the conductors 86 and 87 by a normally open switch 93. This switch is automatically closed upon closing of the main switch 85 by a relay coil 94 which is connected between power lines 82 and 83 by the conductor 87 and a conductor 95.

The pressure valve 51 and the exhaust 63 are operated by solenoids 96 and 97 respectively, each valve being spring retracted to closed position upon the deenergization of the associated solenoid. The solenoids 96 and 97 are formed with a common terminal connected by lead 98 to the conductor 95 and the power line 82. The other terminal of solenoid 96 is connected to the line 83 by a shunt circuit comprising the conductors 99, 100, contact 101, switch arm 102, movable between contact 101 and 103 conductors 104 and 105. The other end of the solenoid 97 is connected to the power line 83 by a shunt circuit comprising conductor 106, contact 103, switch arm 102, and conductors 104 and 105.

The pressure valve 54 and the discharge valve 62 for operation of the piston 25 are actuated by solenoids 107 and 108 respectively, each valve being spring retracted to its closed position. Solenoid 107 is connected to the power line 82 by the conductor 109 and to power line 83 by a shunt circuit comprising the conductor 111 including

the micro switch 45, conductor 112, contact 113, switch arm 114 and conductors 115 and 105. Solenoid 108 is connected to the power line 82 by the common conductor 109 and to line 83 by a shunt circuit comprising conductor 116, contact 110, switch arm 114, conductor 115 and conductor 105.

A control circuit which is connected to the power lines 82 and 83 comprises the conductor 117, the switch 118 operated by the foot pedal 119 as best seen in Figures 1 and 2, conductor 121, and conductor 122 in which is disposed the relay coil 123.

Another control circuit which is also closed by the foot operated switch 118 and is arranged in parallel with the control relay circuit of the relay 123 comprises conductors 117, 121 and 124, anode 125, and cathode 126 of a rectifier tube 127, conductor 128, relay coil 129, anode 131 and cathode 132 of a gas trigger tube 133, and conductors 134 and 105. The filament 135 of the rectifier tube 127 is connected to the power line 82 by conductors 137, and 95, and to the line 83 by conductors 136 and 105. The effect of the rectifier tube is to impress a direct current potential upon the relay coil 129 and the anode 131 of the trigger tube 133.

Current flow from anode 131 to cathode 132 of the gas trigger tube 133 occurs upon charging of the grid 138 to a predetermined value, the resistor 139 limiting current flow from the grid 138 to cathode 132. The grid is charged with a positive voltage to the prescribed value of an R. C. voltage accumulator circuit 141 connected between the cathode 126 of the rectifier tube 127 and the conductor 105. This circuit includes a filtering circuit 142 for filtering the same and the circuit of the relay 129. As usual this accumulator circuit comprises resistance and condenser elements as shown, the time interval required for the voltage build-up being regulated by the variable resistor 143. Discharge of the R. C. circuit is provided for by a discharge circuit comprising the conductor 144 in which is interposed the usual resistance element 145 having a contact terminal 146 adapted to be engaged by switch arm 147.

When the switch 118 is closed, the relay 123 is energized and moves switch arm 102 into engagement with contact 101, connecting conductors 100 and 104 to complete the circuit by which the solenoid 96 is energized for the operation of the valve 51.

Energization of relay coil 123 also moves the switch arm 147 out of engagement with the contact terminal of the resistor 145 to open the discharge circuit 144 thereupon the accumulator circuit 141 begins to charge. When the accumulator circuit is charged with the predetermined voltage the grid 138 actuates the trigger tube 133 allowing current to flow from the anode 131 to cathode 132 to energize the relay coil 129.

Energization of the relay coil 129 moves the switch arm 148 out of engagement with the contact 149 whereby de-energizing relay coil 123. De-energization of the relay coil 123 causes the switch arm 102 to be moved into engagement with the contact 103 to electrically connect conductor 106 with conductor 104 to complete the circuit for energization of solenoid 97 for the operation of the valve 63. Energization of the relay coil 129 also causes switch arm 114 to engage the contact 113 to electrically connect conductor 112 with conductor 115 and thus energize the solenoid 107 which opens the pressure valve 54 for the low-

ering of the tool operator 15. When the switch 148 is opened the relay 129 is de-energized and the switch arm 148 again engages the contact 149. The de-energization of the relay 129 also causes the switch arm 114 to be moved into engagement with contact 110 to connect conductor 116 with the conductor 115 and thus complete the circuit for energization of the solenoid 108 for opening the discharge valve 62, resulting in the elevation of the tool operator 15.

The microswitch 45 is in closed position when the heater element 43 is in its lowermost position and opens at the initiation of the upward movement of this heater in response to opening of the valve 62. The microswitch 45 is interposed in the conductor 111 and prevents operation of the solenoid 107 in response to closing of the switch 113, 114 until the heater 43 has reached the lower limit of its travel.

A switch operator, which is shown on the panel 81 at 153 operates a normally closed switch 154 interposed in conductor 109 and a normally closed switch 155 which normally short circuits a high resistance element 156 of the voltage accumulator circuit 141. The operator 153 in one position closes the switches 154 and 155 for normal operation of the machine. When the operator 153 is thrown to its other position, switches 154 and 155 are opened, having the effect of preventing movement of the tool operator 15 and increasing the time interval required to charge the grid 138 sufficiently for passage of current from anode 131 to cathode 132 of the gas trigger tube 133.

The machine, as disclosed in our said copending application, is also designed for dimpling "Dural" or other metals which may be worked cold, without the development of structural weakness. A switch operator mounted on the panel 81, and indicated in Figure 2 by the numeral 157, operates four switches which appear on the wiring diagram of Figure 3 and are designated by the numerals 158, 159, 161, and 162. Switch 158 is interposed in conductor 95 and when open prevents energization of the relay coil 94 which controls the heater circuit. Switch 159 has two positions, designated on the diagram as M and D. When this switch is in position M conductor 115 is connected to conductor 105 permitting operation of the pressure valve 57 and discharge valve 63. When it is in position D it short-circuits the voltage accumulator discharge circuit 144, connecting this circuit through conductor 163 to conductor 105.

Switch 161 has two positions, indicated by the letters M and D. When in the position M conductors 99 and 100 are connected completing the circuit for operation of the valve 57. When in position D conductor 111 is connected to conductor 100 through a cross-circuit conductor 164 for energization of solenoid 107 for the operation of pressure valve 54 to lower the tool operator.

Switch 162 has two positions, designated by the letters M and D. When this switch is in position M the circuit for the solenoid 97 is complete and the discharge valve 63 may be operated to retract the heating elements to their normal positions. When this switch is in position D it connects conductor 116 with conductor 106 through the cross-circuit conductor 165, completing a circuit for the operation of solenoid 108, which actuates discharge valve 62 for the elevation of the tool operator.

When the switch operator 157 is turned to the lefthand position, as shown in Figure 2 and designated Dow, switch 158 is closed and switches

159, 161, and 162 are in their M position. When the switch operator 157 is in the right-hand position, designated Dural, switch 158 is open and the other three switches are in their D position.

The dimpling dies may be any form desired and the heating elements, as above described, are preferably annular in form for encirclement of the dies. As disclosed in our previously filed application Serial No. 457,630, now U. S. Patent No. 2,372,516, the work contacting faces of the elements are preferably formed of pure silver. The silver has the combination of high specific heat, high conductivity and non-oxidizing qualities, which makes it extremely practical as a contact facing.

The fluid pressure for the actuation of the tool operator 15 should be closely regulated by valve 73 in correlation with the regulation of the temperature of the heating elements. Excessive pressure at a given temperature of the metal sheet may cause thinning of the dimpled and adjacent areas or other deformation of the sheet. Insufficient pressure at a given temperature may result in incompletely formed dimples. This relationship of pressure and temperature may have the following theoretical explanation:

Magnesium and its alloys, particularly aluminum and zinc containing alloys, do not readily lend themselves to cold forming. It is well known that the hexagonal magnesium crystals exhibit fewer slippage planes than crystals of metals which crystallize in more highly symmetrical forms. At temperatures below 410° F. slippage occurs only on the basal planes, while at temperatures above 410° F. pyramidal slippage occurs and plasticity increases very markedly.

It is, therefore, possible to hot work magnesium and its alloys if the workpiece is heated to a temperature above that temperature at which pyramidal slippage comes into operation, but less than that temperature at which the metal will be thinned or will be caused to flow by a minimum effectively sufficiently flexural forming pressure. The critical slippage point, that is, that temperature below which these metals will not yield under pressure along both pyramidal and basal planes without fracture, will of course vary with alloys of different magnesium content.

Forming the metal sheet at a lower temperature and at a correspondingly higher pressure has an additional advantage for certain job requirements. Higher forming pressures of a percussive character have a work hardening effect on the metal. Where this work hardening is an advantage in the finished product, it may be accomplished with metals, such as the magnesium alloys herein described, by adjusting the percussive pressure of the forming tool to a value which is sufficient to work harden the formed zone and heating the metal to a corresponding temperature between points a and c.

The heating elements are designed to have different temperatures, the lower heating element 43 being maintained for example at a temperature preferably of about 650° F. and the upper heater 35 being maintained at a temperature of preferably 900° F. for dimpling the hard rolled magnesium alloy known as Dow metal J, the composition of which is 92.5% magnesium, 6.5% aluminum and the remainder of zinc and manganese. The lower heating element in its normal retracted position is spaced relatively close to the sheet of magnesium metal and the

upper heater is spaced relatively distant therefrom. The heating face of the lower element 43 is also preferably greater in area than the heating face of the upper heating element 35. The capacity of each heater is sufficient to maintain its heating surface at its prescribed temperature.

As a result of these relative heating capacities, heating surface areas, and spacings from the metal sheet, the two heating elements, while held in their retracted position, will, by radiation and to some extent by convection of air currents, heat the metal sheet, although to a degree substantially less than 650° F., the upper heating element contributing to a substantially lesser extent to this heating action.

As the heating elements are moved into and out of contact with the sheet to successively dimple a row of rivet holes, the temperature of the area surrounding any given rivet hole will rise as the operator moves it toward the dimpling dies, reaching a temperature in the example above stated of 650° F., or nearly that temperature, when it is between the dimpling dies.

When at this juncture the heating elements are moved into contact with the metal sheet, the upper heating element acts to bring the temperature of the metal sheet rapidly to the optimum working temperature in a relatively few seconds. In the operation of the machine to carry out the method of the present invention, after a metal sheet is initially heated prior to the first dimpling operation thereon, it requires as little as two seconds of contact of the heating elements with the sheet for bringing that portion of it surrounding a rivet hole to proper working temperature. The upper heater will not overheat the metal in this brief time interval, since the lower heater, being heated to a temperature less than that of the upper heater and being of larger size and having a silver facing, will absorb heat from the upper heater and inhibit a rise in the temperature of the metal sheet.

After the temperature of the heating elements has been regulated to those values suitable for heating a given material to forming temperature, the variable resistor 143 is adjusted to provide a time interval of contact of the heating elements with the sheet which will give the sheet optimum temperature for the desired forming operation.

It is important in the method of the present invention that the sheet be brought accurately to this temperature. If, for instance, the operation is that of dimpling and the adjustment provides too high a temperature, the dimples will be indented too deeply and the sheet will warp. If the temperature is too low, the sheet will develop cracks around the dimple.

A thermocouple (not shown) is embedded in the silver facing of each heating element. Referring to the wiring diagram of Figure 3, the thermocouple of the upper heating element is connected by conductors 169 and 171 to the terminals on one side of a double-throw switch 172. The thermocouple of the lower heater is connected by conductors 173 and 174 to the terminals on the other side of this switch. The movable arms of this switch are connected by conductors 175 and 176 to an electric temperature meter 177. The movable arms of the switch 172 are held by a spring normally in engagement with the terminals of the conductors 173 and 174, since it is more important in the method therein disclosed that the operator have indicated the

temperature of the lower heater. This is true because, as has been explained above, this heater is normally maintained at a temperature less than the upper heater and as it absorbs heat from the sheet the temperature thereof will more closely approximate the temperature of the sheet. When the operator desires to check the temperature of the upper heater he may do so by throwing the switch 172 to connect conductors 169 and 171 with conductors 175 and 176 leading to the meter 177.

The heating elements 35 and 43 are so constructed and secured in place that they are readily removable, the flexible cable leading thereto being provided, as shown in Figure 1, for that purpose with jacks at 178 and 179. This feature of construction of the machine is of advantage in the method herein disclosed for it makes it possible to change the heating elements, using for metal sheets of different thickness and of different curvature, heating elements of corresponding character.

The control box 77, as shown in Figure 2, carries the operator 181 for the switch 162 for selectively connecting the thermocouples of the heaters with the temperature meter 177, which is also mounted in the control box. The lamp 84 is mounted on the panel 81, which also carries the operating lever 183 of the line switch 85, the manipulating knob 184 of the variable resistor 143, as well as the switch operators 153 and 157.

In carrying out the method of the present invention on the machine herein disclosed for dimpling magnesium alloy, the knob 157 is turned to the "Dow" position and the operator 183 manipulated to close the line switch 85. Closing of the line switch 85 lights the beacon lamp 84 and energizes the heating circuit relay 94 which close switch 93 to pass current through the heaters 43 and 45. The temperature of the heaters is regulated by adjustment of the transformer 88 through manipulation of the transformer manipulating knob 92. Since the two heaters are connected in parallel, the temperature of the heaters are proportionately raised or lowered together. However, the heaters may be connected, so that the temperature of the one heater may be regulated without affecting the temperature of the other heater.

A sheet of magnesium alloy is now placed in the machine with one of the rivet holes therein placed upon the usual pilot of the lower die, radiation from the lower heating element, and to a lesser extent from the upper heating element, causing a substantial elevation of the temperature of the metal sheet. Closing of the line switch 83 also sends current through filament 135 of the rectifier tube 121. If, as is usually the case, it is desired to preheat the metal before dimpling the first rivet hole in the sheet, switch operator 153 is temporarily thrown at this time, opening switches 154 and 155.

Upon depression of the foot lever 119 to close the switch 118, current flows to the control relay 123 which connects the circuit leading to the pressure valve 57 and opens the switch in discharge circuit 144. Current now flows through conductor 98 to the solenoid 96, actuating pressure valve 57 operating the piston in cylinder 37 and the piston in cylinder 40 to bring the heating elements in contact with the metal sheet. While the heating elements are held against the metal sheet by valve 57, voltage is being built up in voltage accumulator circuit 141, and at the end of a time interval, which may be regulated for example at two seconds by adjustment of the

knob 184, the gas trigger tube 133 is conditioned for passage of direct current from the rectifier tube 127 through the relay coil 129. When this coil is energized switches 148 and 149 are opened de-energizing coil 123, switch arm 114 engages contact 113 connecting conductors 112 and 115, and disconnecting conductors 116 and 115. De-energization of relay coil 123 connects conductors 106 and 104 to energize solenoid 97, actuating discharge valve 63 to withdraw the heating elements to their retracted position.

De-energization of coil 123 also returns switch arm 147 to the terminal contact 146 of the resistor 145 permitting discharge of the R. C. circuit 141 through the discharge circuit 144 resetting this circuit for the next energization of relay coil 129. The gas trigger tube 133, as is evident from the above, allows energization of relay coil 129 to hold the heating elements in contact with the metal sheet for a prescribed time interval which is unaffected reactively by the movements of the pneumatically energized devices or the flow of current through the solenoids which operate these valves. This electronic control of the heating time interval has a definite advantage over a mechanical, pneumatic or other type of time control. It is highly accurate and is unaffected by the vibration or jars which unavoidably attend the operation of the machine.

When the lower heating element closes the microswitch 45, and assuming that the switch as controlled by operator 153 have been opened, the circuit which energizes solenoid 107 is completed except for the switch 154 which is held open by the operator 153. Since the operator also is holding switch 155 open, the time interval for conditioning the gas trigger tube 133 for passage of current from its anode 131 to its cathode 132 for the energization of control relay coil 129 is lengthened by several seconds, for example 5 seconds. Therefore, as long as the operator 153 holds switch 154 and switch 155 in open position, the dimpling gun assembly will not operate and the heating phase of the operative cycle will be lengthened.

When the sheet is brought close to dimpling temperature, the operator 153 is moved to close switches 154 and 155, shortening the time interval of contact of the heating elements with the metal sheet and closing the circuits to the dimpling gun solenoids 107 and 108. When the control relay coil 129 is energized by operation of the gas trigger tube 133, the lower heating element 43 will close the microswitch 45 completing the circuit to solenoid 107 for the actuation of pressure valve 54 to lower the tool operator. When the tool operator comes into contact with the metal sheet, if it is of the one-shot type, it will deliver its percussion blow to the upper dimpling die upon development of the prescribed pressure against the metal sheet and if it is of the rattle type it will deliver a succession of blows in the manner characteristic of percussion tools of this kind.

The operator now lifts his foot from the foot lever 119, opening switch 118 which breaks the circuit to relay 129. De-energization of relay 129 closes the circuit to solenoid 108 which then actuates the valve 62 to permit the spring 27 to elevate the tool operator 15 to its retracted position. De-energization of relay 129 also, as described above, closes switches 148 and 149 which resets the circuit to relay 123 for its energization, when the operator shall again close foot operated switch 118. In using the machine the operator releases the foot pressure on the pedal

119 to raise the tool operator at the completion of each dimpling operation and again depresses pedal 119 after he has moved the metal sheet to bring the next rivet hole into position for the next dimpling operation, whereupon the cycle is repeated.

While the value of the fluid pressure causing movement of the heating elements into contact with the metal sheet may vary substantially without disadvantage, it should not be so great as to injure the metal sheet nor so small that the heating faces of the elements will not contact the metal sheet with sufficient firmness to provide free conduction of heat from the heating element to the metal.

If desired, the machine may be adjusted to hold the heating elements stationary in their retracted position and the heat within the dies which is received from the encircling heating elements relied upon to raise the metal sheet to proper forming temperature at the time the dies contact the sheet when brought into forming position. To successfully carry out this method the heating elements must be maintained at a higher temperature for any given forming pressure than their temperature when used in the contact method above described and also the dies must be made of a material which will not lose hardness or other qualities desirable in die forming work, at the temperature required to thus bring the metal sheet to forming temperature. Preferably the material of the die should be relatively non-oxidizable at such a temperature and of high specific heat and high thermal conductivity.

The expression "heating element" or "heating body" as used herein is not to be limited to an electrically heated element or body, except where modifying or amplifying context implies such a limitation. The expression defines a body or member which has or is associated with heat delivering means whereby its temperature may be raised, whether that means be an electric current conductor, a heated fluid like steam, or other

means.

While there have been described herein certain embodiments of this invention, the invention is not to be understood as confined to these particular embodiments, for it is susceptible to changes in form and detail within the scope of the following claims.

We claim:

1. A method of dimpling between pressurally related forming elements sheets of a material 55 which cannot be satisfactorily formed below its critical slippage point which comprises: radiationally preheating a preselected local portion 60 of a sheet of said material by mounting the sheet between two heating elements held at different degrees of heat with the portion to be dimpled in sufficiently close proximity to the elements as to receive radiant heat therefrom; moving said elements into engagement with the opposite surfaces of the sheet at the local portion thereof to conductively heat said portion; removing said elements from contact with the opposite surfaces of the sheet; and thereafter applying sufficient percussive flexural force at the center of the heated local portion to properly flexurally form the material without appreciably thinning the same or causing it to appreciably flow.

2. A method of dimpling between pressure applying elements sheets of a material which 75 cannot be satisfactorily formed below its critical slippage point which comprises: pre-heating a

preselected local portion of a sheet of said material to be dimpled by mounting the sheet between two heating elements of annular form held at different degrees of heat with the portion of the sheet to be dimpled in close proximity to the element of the lower temperature; moving said elements into engagement with the opposite surfaces of said portion of the sheet to be dimpled; holding said elements in engagement with said opposite surfaces until the portion of the sheet to be formed is heated to a temperature between the critical slippage point of the material and the degree of heat at which the material will flow even when subjected to a minimum effectively sufficient forming pressure; withdrawing said elements from contact with said surfaces of the sheet and moving said pressure applying elements coaxially of one of said heating elements into pressural engagement with said heated portion; and thereafter applying sufficient pressure to said heated portion to properly flexurally form the material thereof without appreciably thinning the same or causing it to appreciably flow.

3. A method of dimpling between pressure applying elements sheets of a material which cannot be satisfactorily formed below its critical slippage point which comprises: pre-heating a preselected local portion of a sheet of said material to be dimpled by mounting the sheet between two heating elements held at different degrees of heat with the portion to be dimpled in close proximity to the element of the lower temperature; moving said elements into engagement with the opposite surfaces of the sheet with the elements substantially surrounding the local portion of the sheet to be formed; holding said elements in engagement with opposite surfaces of said sheet until the cooler element reaches a temperature greater than the critical slippage temperature of the material but not greater than the temperature at which the material will flow when subjected to a minimum effectively sufficient flexural forming pressure; and thereafter applying sufficient percussive force substantially to the center of the portion heated to flexurally form and harden the material of said portion without causing it to appreciably flow.

4. A method of dimpling sheets of material which has a critical slippage point, comprising: applying heat to opposite surfaces of a preselected local portion of a sheet of said material to quickly raise the temperature thereof; applying flexurally forming pressure to said surfaces; increasing the magnitude of said flexurally forming pressure while continuing said application of heat and so correlating said heat to the melting point of said material as to inhibit warping and burning of said material; and suddenly triggering upon said heated portion a dimpling force of a magnitude predeterminedly so correlated to the critical slippage and flow points of the material of said sheet, and to the then existing temperature of the material of said portion, as to effect sharply defined dimpling of the same, free from fractures, without appreciably thinning or flowing said material.

5. A method of dimpling sheets of a material which has a critical slippage point, comprising: pre-heating a preselected local portion of a sheet of said material by placing said portion between superimposed heating means; moving said heating means into engagement with the opposite surfaces of said portion to quickly raise the temperature thereof; applying oppositely directed flexurally forming pressures to said surfaces; increasing the magnitude of said flexurally forming

pressures while continuing the heating of said material and so correlating the temperature of said material to the melting point thereof as to inhibit warping and burning of said material; and suddenly triggering upon said heated portion a dimpling force of a magnitude predeterminedly so correlated to the critical slippage and flow point of the material of said sheet, and to the then existing temperature of the material of said portion, to form a sharply defined dimple, free from fractures, without appreciably thinning or flowing said material.

6. A method of dimpling sheets of a material which has a critical slippage point, comprising: pre-heating a preselected local portion of a sheet of said material by placing said portion between a pair of spaced heated bodies; moving said heated bodies into engagement with opposite surfaces of said portion to quickly increase the temperature thereof; applying flexurally-forming means to said surfaces; increasing the pressure of said forming means on said surfaces to a predetermined value while continuing application of heat and so correlating said heat to the melting-point of said material as to inhibit warping and burning of said sheet; and suddenly triggering upon said heated portion, by the advent of said value, a dimpling force of a degree predeterminedly so correlated to the critical slippage point and flow point of the material of said sheet, and to then-existing temperature of the material in said minute portion, as to effect sharply-defined dimpling of same, free from fractures, without appreciably thinning or flowing said material.

7. A method of dimpling sheets of a material which has a critical slippage point and is readily combustible and warpable, comprising: pre-heating a preselected local portion of said sheet by placing the same between superimposed heating means with the lower surface in close proximity to the lowermost heating means, the temperature of which is less than the temperature of the uppermost means; applying said heating means to opposite surfaces of the preselected local portion thereby transferring heat from the upper heating means through the sheet into the lower and cooler heating means at a rate sufficient to quickly raise the temperature of the preselected local portion while inhibiting rise in the temperature of the sheet above the temperature of the lower heating means; applying flexurally-forming means to opposite surfaces of the sheet at said portion; increasing the pressure of said forming means on said sheet until the preselected local portion is raised to a temperature between that at which fractures occur in said material when the same is worked and that at which the material will thin or will flow when subjected to the minimum effective forming pressure; withdrawing said heating means from engagement with said preselected local portion; and suddenly causing said forming means to apply a predetermined percussive force to said preselected local portion of a magnitude and time of application so correlated to the critical slippage point and flow point of the material, and to the then existing temperature of said preselected local portion, as to flexurally sharply dimple the portion free from fracture while leaving the portion in an unflowed condition.

GEORGE D. RECHTON.  
DELBERT J. WARD.  
JACK H. WATSON.

## REFERENCES CITED

The following references are of record in the file of this patent:

## UNITED STATES PATENTS

| Number    | Name            | Date           |
|-----------|-----------------|----------------|
| 2,064,232 | Schmidt et al.  | Dec. 15, 1936  |
| 2,247,979 | Von Tanneberg   | July 1, 1941   |
| 2,257,267 | Lundgren et al. | Sept. 30, 1941 |
| 2,288,378 | Veit            | June 30, 1942  |

## FOREIGN PATENTS

| Number  | Country       | Date          |
|---------|---------------|---------------|
| 511,106 | Great Britain | June 30, 1942 |

## OTHER REFERENCES

|                                                                                               |
|-----------------------------------------------------------------------------------------------|
| P. 25 of "Aeronautical Sciences," vol. 8, No. 1, Nov. 1940.                                   |
| Metals Handbook, 1939 ed., pub. by Amer'n Soc. for Metals, 7016 Euclid Ave., Cleveland, Ohio. |